

## UNITED STATES PATENT OFFICE.

GUSTAV F. GERDTS, OF BREMEN, GERMANY.

## METHOD OF TREATING METALS.

No Drawing.

Application filed January 13, 1923. Serial No. 612,517.

*To all whom it may concern:*

Be it known that I, GUSTAV F. GERDTS, citizen of the Republic of Germany, residing at Bremen, Germany, have invented new and useful Improvements in Methods of Treating Metals, of which the following is a specification.

My invention relates to a method of producing metal castings subject to varying strains, use being made of a low grade basic metal or a low grade basic metal alloy. For example, in casting bearings the alloys differ according to the character of the load to which each bearing is to be subjected, so that all plants are compelled to have in stock a large quantity of different kinds of metal which frequently differ from each other in but a small percentage of one or more constituents in order that the required metal for any given use may be on hand. These metals are generally poured out of retorts in which, experience has shown, the metal in most cases is so overheated that a large part of the most valuable constituents burn out and the casting is then not capable of withstanding the load put thereon in actual use. Even in pouring the metal out of crucibles it is difficult to avoid burning as a result of overheating, because the temperature for pouring must be higher than the fusing temperature in order to secure complete castings, but so far as I am aware there are no simple suitable means in existence for precisely determining this temperature.

According to the present invention however, only low grade basic metal is used and this low grade metal is made adaptable for producing bearings capable of sustaining substantial loads by adding to a definite quantity, by weight, of the fused basic metal an addition body which contains the required constituents for producing the desired greater homogeneity or other property of the metal. To these addition bodies other substances may be added which without having the property of modifying the casting may so increase the fusing or melting point of the individual addition bodies that the fusion thereof at the same time gives an indication of the time for pouring whereby overheating of the molten metal is safely avoided.

For example, according to my invention, for the purpose of producing or casting bearings subject to greatly varying loads it is necessary to have in stock only hard lead alloy which suffices for bearings subject to very low load and is made adaptable for higher load bearings by the addition thereto of the corresponding addition bodies. The addition bodies are designated to correspond with the fusion metal or basic metal in connection with which they are adapted to be used to give the correct constitution or the correct temperature for pouring, while for the use of the basic metal alone only addition bodies are employed which do not affect the molten metal but simply, by their fusion, indicate the correct pouring temperature and are so designated.

I am, of course, aware that it is very common in foundry practice to change the character of a metal or of an alloy by adding another metal thereto. But I believe I am the first to make it possible for an ordinary unskilled workman to adapt low grade or basic metal for any desired purpose and to determine the precise temperature at which the molten metal is to be poured. It is not always possible for a skilled foundryman to predetermine the proper pouring temperature of the molten metal, and the usually adopted expedient of immersing a bar of wood in the metal is unreliable because of the varying degrees of moisture of the wood.

By means of the present invention any workman, without previous training in foundry practice or metallurgy, is enabled to adapt a low grade metal or alloy for any desired purpose and by the use of the addition bodies which form the required alloy the precise prescribed pouring temperature is indicated.

The following example will serve to demonstrate the application of the invention in practice.

Assuming that in a shop or factory four different kinds of bearing are in use as follows:—

1. Ordinary bearings for light loads.
  2. Bearings for medium loads
  3. Bearings for heavy loads (bearings for propeller shafts)
  4. Bearings for railway carriages, etc.
- and for these bearings the following four al-

loys, with the indicated ball pressure hardness and melting points, are used:—

| 5<br>No. | Alloy. |    |    | Ball pressure hard-ness. | Metl. point, °C. |
|----------|--------|----|----|--------------------------|------------------|
|          | Pb     | Sb | Sn |                          |                  |
| 10<br>1  | 85     | 15 | 2  | 17                       | 267              |
| 2        | 82     | 16 | 4  | 19                       | 275              |
| 3        | 80     | 16 | 7  | 21                       | 275              |
| 4        | 76     | 17 | 7  | 26                       | 278              |

It would ordinarily be necessary to keep these four alloys constantly on hand to prevent disturbance or stoppage of operation. According to my invention it is merely necessary to have on hand a supply of alloy number 1 to serve as a basic metal, because by adding thereto the proper addition body, alloys numbers 2, 3 and 4 are automatically produced. For alloy number 1 an addition body would be used which does not modify the metal and merely indicates, when it melts, the proper pouring temperature of the molten metal. The following table shows the composition, the melting point and the approximate size of the addition bodies.

| 30<br>No. | Alloy. |      |    | Melt. point, °C. | Size, 0. | mm. high. |
|-----------|--------|------|----|------------------|----------|-----------|
|           | Pb     | Sb   | Sn |                  |          |           |
| 1         | 1.95   | 0.55 | —  | 350              | 25       | 5         |
| 2         | 1.6    | 2.07 | —  | 400              | 31       | 7         |
| 3         | 2.0    | 4.27 | —  | 360              | 37       | 8         |
| 4         | 4.0    | 7.85 | —  | 370              | 44       | 11        |

35 If there be added to the basic metal, per kg., an addition body as above the desired alloy will be obtained. For example, by adding to one kg. of the basic metal an addition body 3 the resulting alloy will correspond exactly to the alloy 3 in the first table, and at the same time the melting of the addition body indicates precisely the proper pouring temperature which, in this case, is 360° C., i. e. 85° higher than the melting temperature of alloy number 3. Thus unintentional or accidental overheating is guarded against.

The addition body 1 indicates only pouring temperature, about 80° higher than the melting temperature of alloy number 1, while the melting temperature of the addition body number 3 is about 90° higher than the melting temperature of the alloy number 3 and thus serves, per se, as an index to the pouring temperature. The melting point of addition body number 2 is 400° C. and, in order that this temperature may be only about 80° higher than the melting temperature of alloy 2, the addition body 2 has added thereto a small quantity of a metal (such as bismuth) which lowers the melting temperature to about 360° C. but

but which, by reason of the small quantity used, does not affect the properties of the basic metal. In the foregoing table the addition bodies are indicated by numbers 1 to 4, but even without these numbers the bodies could be distinguished from each other because of their difference in size, the increasing in size from number 1 to number 4 being uniform.

The procedure according to my invention is very simple and requires no special attention on the part of the operator. As soon as the basic metal has been melted, the slag layer is removed from the middle of the crucible of fusion chamber and the addition body is laid on the fluid metal bath, such addition body corresponding to the load which the casting is to withstand. As soon as the addition body has melted the entire mass is stirred and then immediately poured, because when the addition body melts the correct temperature for pouring is reached.

To prevent oxidation of the surface of the metal bath, the addition bodies may be combined with a de-oxidizing mass, such as alkali carbonate, borax, etc., which immediately upon contacting with the hot surface of the metal melts and covers the latter. This protective mass may be enclosed by the addition body like a capsule or may partly or entirely enclose it, in order to protect the addition body against oxidation.

#### Claims:

1. The herein described method of adapting low grade metal to desired uses, which consists in adding to the molten metal for each given unit of weight thereof a metal addition body which, when it melts, indicates the correct pouring temperature of the molten metal.

2. The herein described method of adapting low grade metal to desired uses, which consists in adding to the molten metal for each given unit of weight thereof a metal addition body which imparts improved qualities to the molten metal and which addition body, when it melts, indicates the correct pouring temperature of the molten metal.

3. An addition body for low grade metals, comprising a metal alloy having a melting temperature indicative of the proper pouring temperature of the molten metal to which the addition body is added.

4. An addition body as claimed in claim 3 combined with a de-oxidizing protective mass.

In testimony whereof I have affixed my signature.

GUSTAV F. GERDTS.

#### Witnesses:

FRANCIS J. DUGAN,  
AUGUST QUICK.